

**1**

3,677,975

**PREPARATION OF SOLID SOLUTIONS OF METALLIC OXIDE MIXTURES BY FLAME-SPRAYING**

John E. Bennett, Painesville, and Kevin J. O'Leary, Cleveland Heights, Ohio, assignors to Diamond Shamrock Corporation, Cleveland, Ohio  
No Drawing. Filed Oct. 26, 1970, Ser. No. 34,111  
Int. Cl. H01b 1/06; B05b 7/20; C22b 11/00  
U.S. Cl. 252—518 **8 Claims**

**ABSTRACT OF THE DISCLOSURE**

A solid solution of a valve metal dioxide and a precious metal dioxide is prepared in bulk form independent of a substrate by passing, in finely-divided atomized form, an organic solution of a salt or ester of the valve metal and a salt of the precious metal through an oxidizing flame.

**BACKGROUND OF THE INVENTION**

A wide variety of solid solutions have long been known and used in the art. Recently, specific types of solid solutions have been developed which are particularly useful as electrically-conducting components in electrolytic applications. These particular solid solutions, composed primarily of mixtures of valve metal and precious metal oxides, are formed when heated in contact with a conductive base as described more fully, for example, in South African Pat. 68/0834. Anodes prepared in accordance with this teaching exhibit properties so superior to prior known and used dimensionally-stable anodes that they have enjoyed ever increasing and widespread commercial use, particularly in chlor-alkali electrolytic processes. Because of the excellent electroconductive and catalytic properties of these anodes, many attempts accordingly have been made in the art to adapt the solid solutions on which they are based for use in other related applications.

It has been found, however, that in contrast to the teachings of the aforementioned South African patent, true solid solutions, particularly valve metal dioxide-precious metal dioxide solid solutions, are obtained only when the component metal oxides are formed in contact with a conductive base. Additionally, it has been found from practice of the aforesaid South African patent teachings, that certain electroconductive solid solutions, e.g., a titanium dioxide-ruthenium dioxide solid solutions can be so formed on only certain selected conductive substrates, preferably titanium. Attempts to form such solid solutions, i.e., polycrystalline materials wherein molecules of titanium in the characteristic tetragonal (rutile) titanium dioxide lattice are randomly replaced with molecules of ruthenium, have not been successfully accomplished on a substrate such as nickel. In contact with this metal, only adherent, physical mixtures of the oxides are obtained, identifiable as separate crystalline phases. Attempts to form titanium dioxide-ruthenium dioxide solid solutions likewise have not been successfully accomplished on lead or other soft metals more susceptible than titanium to deterioration when exposed to elevated temperatures.

Widely known methods for preparing solid solution-type materials in bulk form as set forth, for example, in U.S. Patent Nos. 3,498,931 and 3,514,414, have the disadvantage of requiring the use of sealed reaction vessels, vacuum, high pressure and the like and are best adapted only to small scale operation. A much simpler technique for preparing solid solutions have been developed which requires no such sealed equipment or strenuous

**2**

operating conditions. This method which is described in a pending U.S. patent application, Ser. No. 74,876, filed in the name of James M. Kolb, generally involves slowly heating an intimate mixture of a finely-divided valve metal and a salt of a precious metal in an oxidizing atmosphere for a sufficient time period to convert the valve metal and precious metal to their respective dioxides. With this method, the desired metallic oxidation state typically is attained by heating the aforesaid mixture at a prescribed slow rate up to a temperature of 450°-600° C., which process may involve 24 hours heating time or even longer.

**SUMMARY OF THE INVENTION**

We have now found that a true valve metal dioxide-precious metal dioxide solid solution may easily be obtained in bulk form and independent of a substrate by first

- 15 (a) Preparing a solution of a salt or an ester of a valve metal and a salt of a precious metal; and then  
20 (b) Flame-spraying said solution by passing it through an oxidizing flame maintained at a temperature sufficient to convert both the valve metal and the precious metal essentially to their respective dioxides with the concurrent formation of a solid solution of said metal dioxides.

From the flame zone, the solid solution thus formed may be passed into suitable apparatus wherein it can be collected in particulate form for future use in a variety of applications typically with no further chemical or modifying treatment. It may easily be applied, for example, either alone or in combination with other ingredients onto a conductive and/or supporting base.

- 30 35 Alternatively, of course, the solid solution may be directly sprayed onto a conductive and/or supporting base, forming a hard, tightly bonded and durable conductive coating thereon.

The process of this invention has many distinct and commercially important advantages over all prior art methods for preparing solid solutions of this type in bulk form independent of the metal base. First, this process is a much faster and more economical method than the already known techniques, since the flame-spraying and subsequent product collection or deposition steps together may be effected in a total time period of one several seconds. Also, it is a simple, safe method for forming solid solutions, requiring no expensive equipment and/or hazardous operations as pressure-sealed tubes, inert atmospheres, high vacuum, high pressure, etc. Of utmost importance, of course, is the fact that by practice of this invention, it is possible to prepare valve metal dioxide-precious metal dioxide solid solutions which consistently are of a high degree of purity. Particularly,  $TiO_2$ - $RuO_2$  solid solutions of this invention contain no detectable "free" precious metal dioxide as a separate crystalline phase.

**DESCRIPTION OF THE PREFERRED EMBODIMENTS**

The solid solutions of the present invention are mixtures of oxides of the various valve metals and precious metals. As used herein, the term "valve metals" has the standard connotation and refers to titanium, zirconium, niobium and tantalum metals. The term "precious metal" is intended herein to refer primarily to the platinum group metals: platinum, ruthenium, iridium, palladium, rhodium, and osmium.

65 70 In the practice of this invention, either a suitable ester or salt of the valve metal may be employed. Suitable esters are compounds, preferably liquid, which have the

general formula —Me(OR)<sub>x</sub>— wherein Me is the valve metal; R is a hydrocarbon radical, preferably aliphatic, having from about 3 to 8 carbon atoms; and x is the valence of the metal. In the presently preferred embodiments of the invention wherein titanium is the valve metal, specific esters thereof suitably used include, for example, tetraisopropyl titanate, tetrabutyl titanate, or tetra 2-ethylhexyl titanate. It should be noted, however, that any ester of a valve metal generally may be used providing said ester, if not a liquid, can be easily dissolved in the organic liquid solvating medium which is employed in preparing the mixed metallic solution. Valve metal salts suitably employed include the halides thereof, e.g. TiCl<sub>3</sub>, and other salts which can be decomposed at the flame-spraying temperatures utilized herein.

The precious metals are employed typically in a powdered salt form, e.g., in the form of hydrated halides such as RuCl<sub>3</sub>·2.5 H<sub>2</sub>O, etc., usually for convenience and owing to commercial availability of these materials. However, any decomposable form of the previous metal, e.g., an ester thereof, can be used.

In general, the amounts of the two metallic compounds which may be employed to form the solution subsequently flame-sprayed in the practice of this invention depend, of course, upon the relative amounts of precious metal oxide which the valve metal oxide crystal lattice will incorporate into a solid solution conforming to the formula Y<sub>x</sub>Z<sub>1-x</sub>O<sub>2</sub>, wherein Y=the precious metal and Z=the valve metal. In the case of the RuO<sub>2</sub>-TiO<sub>2</sub> system, the amount of precious metal incorporated generally will vary between 0.01 and 99+%, as the metallic oxide molecules are freely interchangeable in the lattice. Within this range, the amount of ruthenium actually employed is varied depending upon the intended use of the solid solution and economic considerations, use of 20-80% RuO<sub>2</sub> being typical.

In carrying out the present invention, the solution of the precious metal salt and the valve metal compound to be flame-sprayed is prepared in an organic solvating medium such as a lower alkanol, e.g., isopropanol or n-butanol. In practice of presently preferred embodiments herein, the precious metal salt, as RuCl<sub>3</sub>·2.5 H<sub>2</sub>O usually is first mixed with a small amount of a mineral acid, e.g., HCl, to aid its subsequent dissolution in the alcohol. The precious metal salt-acid mixture is then mixed with the alcohol and the metal salt completely dissolves. Thereafter, the valve metal, e.g., titanium compound is dissolved in the precious metal salt solution. After preparation, the metallic solution may immediately be flame-sprayed or, if necessary, may be stored for several hours prior to processing, with equivalent results.

The prepared metallic solution is passed as a finely-divided atomized spray through an oxidizing flame to form the desired valve metal dioxide-precious metal dioxide solid solution. Typically, the solution will be propelled into the ignition zone by a carrier gas, such as air, in admixture with a fuel gas. Aspiration of the solution-gas mixture usually provides impetus to the atomization process. However, any flame-spraying technique now known for flame spraying, e.g., metal powders, may be successfully employed herein.

From the flame zone, the product may be drawn by vacuum into a suitable device such as a cyclone separator wherein it is isolated from the gaseous phase and collected in particulate form. Alternatively, as pointed out previously herein, the solid solution may be sprayed onto a conductive and/or supporting base. In the case of heat-sensitive base materials, such a substrate is positioned at a prescribed distance from the flame so as not to be distorted or otherwise deleteriously affected thereby.

In carrying out the flame-spraying operation, the temperature of the oxidizing flame is quite critical and must be maintained within the range of 900-1600° C., preferably from 1000-1500° C., particularly when forming TiO<sub>2</sub>-RuO<sub>2</sub> solid solutions. If passed through a flame

which is hotter than 1600° C., the metals, especially a precious metal such as ruthenium, will be converted to oxides higher than the desired dioxide. Such higher oxides are, in most instances, vaporous compounds. Conversely, if the metallic solution is aspirated through a flame maintained at a temperature much below 900° C., the desired oxidation state of these metals will not be attained to any significant degree, if at all. Further, if any metal dioxides should be formed, these usually will exist only in separate phases and are easily identifiable as such, no true solid solution being obtained.

As the flame source, any fuel suitably may be employed in an oxygen atmosphere, e.g., in air, providing the heat generated by the fuel-oxidant flame can be controlled within the above-described critical temperature range. To date, mixtures of either natural gas or hydrogen with air have been easily regulated to provide oxidizing flames of the desired temperature. Under the same operating conditions, however, no similar acetylene mixture, whether rich or deficient in air, has been found satisfactory up to the present time. Flame temperatures can conveniently be measured herein by means of an optical pyrometer.

In carrying out flame-spraying operations, the temperature of the oxidizing flame is regulated within the proper range by adjusting the flow rates of the air and fuel streams entering the burner of the flame-spraying apparatus. Typically, when employing hydrogen as the fuel, a flow rate of about 5 to 14 cubic feet of air/hour for each cubic foot/hour of hydrogen will provide efficient oxidant-fuel mixtures.

It is further to be noted that regulation of the oxidant-fuel flow rates likewise serves to provide, in conjunction with the burner head, an oxidizing flame of the proper dimensions, e.g., height, thereby preventing excessive exposure of the sprayed solution to intense heat and conversion of the metal components to undesirable oxides. Depending upon the air-fuel mixtures employed in practice of this invention, selection of burner heads with the proper width can be easily determined with minimum experimentation. When employing air-hydrogen mixtures within the aforementioned flow rates, use of a burner head about 4 inches wide has been found particularly suitable.

The valve metal oxide-precious metal oxide solid solutions of this invention obtained either as powders or as coherent coatings, are electrically conductive materials. These products consistently are highly pure products, as indicated by X-ray analysis of their crystalline structure. In presently preferred embodiments of this invention, wherein titanium and ruthenium respectively are the particular valve and precious metals employed, X-ray diffraction patterns of the solid solutions obtained show these to be essentially rutile form solid solutions of titanium and ruthenium dioxides. No evidence is found indicating the presence of any free precious metal dioxide in these products.

The valve metal oxide-precious metal oxide solid solution products of this invention are useful in a variety of applications. For example, it has been found that electrical resistors of predictable degrees of resistivity are readily formed by varying the relative amounts of valve and precious metal components, the relationship between the mole percent of precious metal present and the electrical conductivity being a reproducible function. This property also makes solid solutions of the present invention useful in the manufacture of capacitors and other electronic components.

The solid solutions have also proven useful as non-specific oxidation catalysts for gaseous phase reactions. The catalytic activity of the solid solutions appears extremely high and use of these materials as exhaust emission control catalysts is suggested.

In addition, owing to their excellent electroconductivity and electrocatalytic activity, the solid solutions are useful in a number of electrochemical applications, especially in view of the fact that they may easily be applied, e.g.,

by spraying, onto a variety of supporting and conducting substrates, which was not true in previous electrochemical applications where their use on a substrate of the parent valve metal was usually dictated. Use in fuel cell applications is particularly promising.

In order that those skilled in the art may more readily understand the present invention and the preferred methods by which it may be carried out, the following specific examples are offered. In these examples where proportions of ingredients used may be expressed in parts, such proportions are by weight.

#### EXAMPLE 1

A solution containing for each part of  $\text{RuCl}_3 \cdot \text{XH}_2\text{O}$  (0.4 part Ru metal), 6.2 ml. n-butyl alcohol, 3.0 ml. tetrabutyl orthotitanate, and 0.4 ml. 36% HCl, is aspirated into an air stream of 32.3 cubic feet per hour. This stream is then combined with 2.66 cubic feet per hour of hydrogen and ignited at a burner head 4 inches wide to produce a dull orange flame. The products of the flame are passed through a cyclone where the solid oxides produced are separated from the gases present.

Product thus collected is an electrically conductive black powder. It is shown by X-ray analysis to be a substantially pure rutile form solid solution of titanium and ruthenium dioxides, providing only one X-ray reflection from each crystallographic plane. In contrast, mixtures of these dioxides in free form provide interplanar spacings corresponding to each separate crystalline phase. Interplanar spacing of the 110 crystal plane for the product is 3.20 Å. as compared to 3.18 Å. for free ruthenium dioxide and to 3.245 Å. for free titanium dioxide.

#### EXAMPLE 2

A solution prepared as in Example 1 is again aspirated into an air stream of 32.3 cubic feet per hour. This stream is then combined with 5.07 cubic feet per hour of hydrogen and ignited at a burner head to produce a light orange flame.

Product collected as in Example 1 is again an electrically conductive black powder indicated by X-ray analysis to be a substantially pure rutile form solid solution of titanium and ruthenium dioxides. Interplanar spacing of the 110 crystal plane for this material is 3.22 Å.

In contrast to the foregoing examples, flame-spraying of identical metallic solutions under similar conditions using various air-acetylene mixtures as the oxidant-fuel flame source did not produce the desired solid solutions. The products thus obtained were nonconductive powders grayish in color. These products were found, by X-ray analysis, to be predominantly mixtures of anatase and

rutile titanium dioxide. No ruthenium dioxide was found to be present, even in separate crystalline phase.

While the invention has been described with reference to certain preferred embodiments and techniques, it is not to be so limited since changes and alterations may be made therein which are fully within the intended scope of the appended claims.

We claim:

1. A method for preparing a valve metal dioxide-precious metal dioxide solid solution in bulk form independent of a substrate which comprises:
  - (a) preparing a solution of an ester or a salt of a valve metal and a salt of a precious metal;
  - (b) flame-spraying said solution by passing it through an oxidizing flame maintained at a temperature sufficient to convert both the valve metal and the precious metal essentially to their respective dioxides with the concurrent formation of a solid solution of said metal dioxides.
2. The method of claim 1 wherein the valve metal is titanium and the precious metal is ruthenium.
3. The method of claim 2 wherein the ruthenium metal is present in the solid solution in the range of 20-80%, on an  $\text{RuO}_2$  basis.
4. The method of claim 1 wherein the solid solution of the valve metal and precious metal dioxides upon emergence from the flame zone is collected in particulate form.
5. The method of claim 1 wherein the solid solution of the valve metal and precious metal dioxides is sprayed from the flame zone onto a supporting base.
6. The method of claim 5 wherein the supporting base is conductive.
7. The method of claim 1 wherein the oxidizing flame is maintained at a temperature ranging from 900° to 1600° C.
8. The method of claim 1 wherein the oxidizing flame is supplied by an air-hydrogen mixture introduced into the ignition zone at a flow rate ratio of 5-14 cubic feet of air/hour for each cubic foot/hour of hydrogen.

#### References Cited

##### UNITED STATES PATENTS

- |    |           |         |                         |         |
|----|-----------|---------|-------------------------|---------|
| 45 | 3,305,349 | 2/1967  | Bovarnick et al. -----  | 75—5 AA |
|    | 3,172,753 | 3/1965  | Walsh -----             | 75—5 AC |
|    | 3,062,638 | 11/1962 | Culbertson et al. ----- | 75—5 BB |

DOUGLAS J. DRUMMOND, Primary Examiner

50 U.S. CL. X.R.  
252—520; 117—221, 105.2; 75—0.5 B, 0.5 BB